

Patented Nov. 8, 1932

1,886,995

# UNITED STATES PATENT OFFICE

HEINRICH WERDENBERG, OF NEU-ALLSCHWIL NEAR BASEL, SWITZERLAND, ASSIGNOR  
TO THE FIRM OF DURAND & HUGUENIN S. A., OF BASEL, SWITZERLAND

## PRODUCTION OF DYEINGS AND PRINTS ON MIXED FABRICS

No Drawing. Application filed March 12, 1931, Serial No. 522,155, and in Germany March 17, 1930.

In U. S. patent application Ser. No. 480,027, filed September 5, 1930, a process for dyeing cellulose ester fibre with gallocyanine dyestuffs has been disclosed. This process is based on the observation that these gallocyanine dyestuffs have in their leucoform a better affinity for the said fibre than in the oxidized form. Therefore it is advantageous to bring a leuco compound of a gallocyanine dyestuff onto the cellulose ester fibre and to develop the dyeing thereon by means of a suitable oxidizing agent.

The application of the above mentioned dyestuff-class on cotton fibre proceeds in a somewhat different manner as the gallocyanines in the form of the dyestuffs themselves as well as in the form of their leuco compounds show an insufficient affinity for the fibre. To realize the fixation thereon, a gallocyanine or its leuco compound is therefore printed or padded on the fibre together with a chromium salt, whereupon the desired dyeing is developed as an insoluble chromium lake by means of steaming.

By these means, however, it is not yet possible to dye or print mixtures of cellulose ester and cotton in a satisfactory manner. The first mentioned dyeing process is suitable for dyeing the cellulose ester fibre, but the cotton contained in the fabric mixture is dyed quite insufficiently. On the other hand the process with chromium salts, such as it is applied to cotton, is quite unsuitable for cellulose esters, as the latter fibre possesses only a very slight absorbing property for the chromium lake which is formed.

Mixed fabrics, however, containing cellulose ester fibre and a cotton fibre, i. e. vegetable cotton or artificial silk being based on cellulose material such as viscose, copper-silk (Bemberg silk) etc., are used actually to a large extent and the dyeing or printing of such fabrics has become an important problem.

It has now been found that it is possible to dye such mixed fabrics evenly with gallocyanine dyestuffs if one works first in an an-

alogous manner to that described in the aforesaid U. S. patent application for pure cellulose ester fibre, that is to say if a gallocyanine dyestuff is brought onto the fabric in the form of its leuco compound, if this fibre is steamed, whereby the fixation of the dyestuff on the cellulose ester fibre takes place, and if afterwards by a treatment with a suitable chromium compound the fixation of the dyestuff on the cotton fibre is performed.

Generally the dyestuff, after the steaming, will be fixed but not developed on the cellulose ester fibre, that is to say, it is found thereon as leuco compound and must be oxidized to the dyestuff. This oxidation and simultaneously the fixation of the dyestuff on the cotton fibre may be performed by an after-treatment of the fabric in an acid bichromate solution.

In the same way as in the process of the aforesaid U. S. patent application, also in the present one, simultaneously with the dyestuff a suitable oxidizing agent, inactive in the cold, active in hot state and incapable of causing the formation of a lake with the dyestuff, may be brought onto the fabric. After steaming the dyestuff is fixed and developed on the cellulose ester fibre and by an after-treatment with a suitable chromium compound the fixation of the dyestuff on the cotton fibre can be performed.

The improved process is illustrated by the following examples.

The following printing pastes are prepared:

### Example I.

|                                         | Parts |
|-----------------------------------------|-------|
| Leuco prune (see Colour Index No. 893)  | 30    |
| Hot water                               | 90    |
| Gum thickening                          | 120   |
| Neutral starch and gum dragon           | 350   |
| thickening                              | 400   |
| Heat up to dissolve, cool down and add: | 95    |
| Turpentine oil                          | 20    |
| Sodium chlorate solution (1:3)          | 80    |
|                                         | —     |
|                                         | 1000  |
|                                         | 100   |

*Example II*

|                                               | Parts |
|-----------------------------------------------|-------|
| Leuco Correine R R (see Colour Index No. 900) | 30    |
| 5 Hot water                                   | 120   |
| Gum thickening                                | 350   |
| Neutral starch and gum dragon thickening      | 400   |
| Heat up to dissolve, cool down and add:       |       |
| 10 Turpentine oil                             | 20    |
| Sodium chlorate solution (1:3)                | 80    |
|                                               | 1000  |

*Example III*

|                                                              | Parts |
|--------------------------------------------------------------|-------|
| 15 Phenocyanine V S in paste form (see Colour Index No. 902) | 100   |
| Cold water                                                   | 50    |
| Gum thickening                                               | 350   |
| Neutral starch and gum dragon thickening                     | 400   |
| 20 Turpentine oil                                            | 20    |
| Sodium chlorate solution (1:3)                               | 80    |
|                                                              | 1000  |

*Example IV*

|                                                                                                                          | Parts |
|--------------------------------------------------------------------------------------------------------------------------|-------|
| Leuco compound of the condensation product from Correine R R with diethylparaphenylenediamine (see Colour Index No. 884) | 30    |
| Hot water                                                                                                                | 120   |
| Gum thickening                                                                                                           | 350   |
| Neutral starch and gum dragon thickening                                                                                 | 400   |
| 35 Turpentine oil                                                                                                        | 20    |
| Sodium chlorate solution (1:3)                                                                                           | 80    |
|                                                                                                                          | 1000  |

40 Print these pastes on mixed fabric of acetate silk and cotton, dry, steam for 1 hour, treat afterwards at ordinary temperature in a bath containing 5 gr. of bichromate of soda per liter of water, and wash. Thus one obtains evenly developed and normal dyeings on both kinds of fibres.

45 In these cases instead of bichromate in an analogous manner another chromium compound such as for instance chromium acetate may be used with a similar result.

*Example V*

|                                             | Parts |
|---------------------------------------------|-------|
| Prune (see Colour Index No. 893)            | 30    |
| Hot water                                   | 342   |
| 55 Hydrosulphite NF conc. (powder)          | 8     |
| Heat up until completely reduced, then add: |       |
| Neutral starch and gum dragon thickening    | 600   |
| 60 Cool down and add:                       |       |
| Turpentine oil                              | 20    |
|                                             | 1000  |

65 Print on mixed fabric, steam for 40 minutes. After steaming treat in a bath contain-

ing 10 gr. of sodium bichromate and 10 ccm. of formic acid (85 per cent) per liter for 10 to 15 minutes, rinse and soap.

When using a printing paste which contains a chromium salt, such as for instance chromium acetate, only uneven and dull shades are obtained, as in this (latter) case the acetate silk fibre is dyed only very slightly.

By the present process, dyeings on mixed fabrics may also be produced by padding.

In this process the gallocyanine dyestuffs may also be used in mixtures with dyestuffs of other classes capable of being absorbed by the cellulose fibre and of being fixed on cotton fibre as a chromium lake such as for instance yellow wood extract.

What I claim is:

1. A process for producing dyeings and prints on mixed fabrics containing cellulose ester fibre and a cotton fibre by means of gallocyanine dyestuffs, which consists in bringing a gallocyanine dyestuff in form of its leuco compound onto the fabric, subjecting the same to a steaming operation, necessary for the fixation of the dyestuff on the cellulose ester fibre, and then after-treating the fabric with a suitable chromium compound to produce fixation of the dyestuff on the cotton fibre.

2. A process for producing dyeings and prints on mixed fabrics containing cellulose ester fibre and a cotton fibre by means of gallocyanine dyestuffs, which consists in bringing a gallocyanine dyestuff in form of its leuco compound onto the fabric, subjecting the same to a steaming operation necessary for the fixation of the dyestuff on the cellulose ester fibre and then after-treating the fabric in an acid bichromate solution, so as to produce simultaneously oxidation of the leuco-compound to the dyestuff and fixation of the dyestuff on the cotton fibre.

3. A process for producing dyeings and prints on mixed fabrics containing cellulose ester fibre and a cotton fibre by means of gallocyanine dyestuffs, which consists in bringing onto the fabric a gallocyanine dyestuff in form of its leuco compound simultaneously with an oxidizing agent, which is inactive in the cold, but becomes active to perform the necessary oxidizing action in hot state, subjecting the fabric to a steaming operation for the fixation of the dyestuff on the cellulose ester fibre and then after-treating same with a suitable chromium compound to produce the fixation of the dyestuff on the cotton fibre.

In witness whereof I have hereunto signed my name this 2nd day of March 1931.

HEINRICH WERDENBERG.

125

130